

## UNITED STATES PATENT OFFICE

2,060,856

## INSULATED ELECTRICAL CONDUCTOR

John M. De Bell, Newark, Del., assignor to  
 Hercules Powder Company, Wilmington, Del.,  
 a corporation of Delaware

No Drawing. Application April 20, 1935,  
 Serial No. 17,471

8 Claims. (Cl. 175—356)

This invention relates to an insulated electrical conductor.

The insulated electrical conductor in accordance with this invention comprises an electrical conductor in combination with an insulating material composed of a resinous composition known as extracted pine wood pitch, which is a residue comprising oxidized resin acids such as abietic acid, oxidized terpenes, polyphenols, polymerized 5 terpenes and frequently some ligneous matter left after the separation of rosin, turpentine and other more valuable constituents of pine wood.

The insulated electrical conductor in accordance with this invention will be found to be 15 highly efficient due to its high dielectric strength, especially under impulse tests, and the insolubility of the extracted pine wood pitch, in oils, as transformer oils.

The pine wood pitch for the production of the 20 insulated conductor in accordance with this invention, as has been indicated, is obtained in connection with the production of wood rosin from pine wood. The pine wood pitch will comprise oxidized resin, oxidized abietic acid, oxidized 25 terpenes, polyphenols, polymerized terpenes, and more or less ligneous matter, but will differ somewhat in its specific characteristics, such as acid number, melting point, petroleum 30 ether solubility and content of naphtha and toluol soluble matter, depending upon the method for the recovery of rosin from pine wood used in its production.

As is well known, rosin is extracted from pine 35 wood by the use of a suitable solvent, such as hot gasoline, or benzol, after steaming of the wood with live steam to remove volatile oils, such as turpentine and pine oil. Again, volatile oils, as 40 turpentine, and pine oil, are extracted with the rosin without first steaming for their removal.

Following extraction the extract is distilled 45 for the removal of solvent where the wood was subjected to steaming before extraction and for the removal of solvent and volatile oils, as turpentine and pine oil, where the wood was extracted directly without steaming. As the result 50 of distillation a resinous material consisting of a mixture of rosin, oxidized abietic acid, oxidized terpenes, polyphenols, polymerized terpenes and ligneous matter is obtained. This resinous material may be treated in any one of a number of 55 ways, all known to the art, for the removal of refined rosin. The residue remaining after the removal of refined rosin and including oxidized abietic acid, oxidized terpenes, polyphenols, polymerized terpenes and ligneous matter originally

present in the extract and comprising a dark colored, hard, resinous mass constitutes the pine wood pitch.

The exact properties of the pine wood pitch obtained as indicated above will depend upon the 5 method used for original extraction from the wood. When the wood is steamed before solvent extraction, a pine wood pitch is obtained having somewhat different properties from that obtained when the wood is extracted without steaming. 10 Likewise the properties of pine wood pitch are somewhat different when obtained by different methods of purification of rosin. A comparison of the properties of three pine wood pitches is 15 given in the following table, in which Pitch A is 20 that obtained by extraction of wood with hot petroleum solvents subsequent to the removal of the volatile oils by steam distillation, refining with furfural, evaporation of furfural to leave a resinous mass and then extraction of this mass with 25 a petroleum solvent to remove petroleum soluble resin. Pitch B is that obtained by a benzol extraction of unsteamed wood, evaporation of the benzol solution of the residue in hot low boiling petroleum solvent, precipitation of the Pitch B 30 by washing with cold water, and then removal of this precipitate by filtration. Pitch C is obtained by the evaporation of the furfural layer, after refining of the gasoline solution of the crude resin obtained by the benzol extraction of pine wood. 35

|                                         | Pitch A | Pitch B | Pitch C |    |
|-----------------------------------------|---------|---------|---------|----|
| Melting point (Hercules drop method)... | 91° C.  | 115° C. | 102° C. | 35 |
| Acid number.....                        | 100     | 105     | 116     |    |
| Unsaponifiable matter.....              | 5%      | 8%      | 8%      |    |
| V. M. & P. naphtha insoluble.....       | 89.5%   | 96%     | 83%     |    |
| Toluol soluble.....                     | 40%     | 40%     | 98%     |    |
| Petroleum ether insoluble.....          | 92.0%   | 99%     | 95%     |    |
| Saponification number.....              |         | 169     | 140     |    |
| Ash.....                                |         | .036%   | .022%   | 40 |

It will be noted that while this extracted pine wood pitch contains oxidized rosin or abietic acid, certain of its properties are entirely different from those of so-called oxidized rosin produced by oxidation of rosin. Thus, for example, extracted pine wood pitch is substantially insoluble in natural petroleum hydrocarbons while oxidized rosin is readily soluble in these solvents.

The insulated electrical conductor in accordance with this invention may include the extracted pine wood pitch alone or in admixture with other substances which may desirably be admixed with it for variation of its physical 55

characteristics, such, for example as wood pitch, copal, coal tar asphalt, small amounts of castor oil, rubber, a rosin residue resulting from the steam distillation of pine oil, etc.

5 The insulated electrical conductor in accordance with this invention may be of any type or form, however, for convenience I will proceed with a more detailed description of this invention with reference to its application to transformer coils in connection with which it is especially advantageous, more particularly in view of its very high resistance to impulse tests and its insolubility in transformer coils.

In the production of a transformer coil embodying this invention, the coil is wound as usual, using any desired insulated wire for the winding and the coil being of any desired form or capacity. After the coil is completely assembled, it is electrically insulated and mechanically bonded 20 in any suitable or well known manner with the extracted pine wood pitch, described above, either alone or in combination with other desired ingredients, such as have been indicated by way of example.

25 By way of example the coil may be insulated and bonded in a well known manner by placing it in a tank, placing the tank under vacuum, running the extracted pine wood pitch in at a temperature at which it will be fluid and then 30 draining off excess pine wood pitch after the desired impregnation has been effected. On cooling, the coil will be found to be efficiently insulated and bonded.

The impregnation may be efficiently accomplished with the extracted pine wood pitch alone or in admixture with other ingredients, at a temperature of about 150° C. to about 165° C.

Where it is not desired to use extracted pine wood pitch alone, mixtures made up on any of 40 the following formulae will be found to be satisfactory:

|                                    | No. 1 | No. 2 | No. 3 | No. 4 |
|------------------------------------|-------|-------|-------|-------|
| 45 Extracted pine wood pitch.....  | 90    | 95    | 90    | 85    |
| Coal tar asphalt.....              | 10    | 5     | 10    | 15    |
| Copal.....                         |       |       |       |       |
| Castor oil.....                    |       |       |       |       |
| Pine oil distillation residue..... |       |       |       |       |

50 In the production of insulated conductors in accordance with this invention, it will be desirable, though not essential, that the pine wood pitch be subjected to heat treatment prior to use alone or in admixture, in order to avoid foaming during the impregnation of a conductor under elevated temperature at which it will be fluid. By way of illustration, the extracted pine wood pitch may desirably be treated at a temperature of from about 150° C. to about 325° C. 55 for a period of from about 10 minutes to about 2 hours, depending upon the temperature. More specifically, the pine wood pitch, if treated at a temperature of about 250° C. for about one

hour, will not foam at impregnating temperatures.

It will be understood that the conductor in accordance with this invention may be of any type and may include insulating material other than and in addition to the extracted pine wood pitch described herein.

What I claim and desire to protect by Letters Patent is:

1. In combination an electrical conductor and an insulating material therefor comprising a pine wood pitch obtained by the extraction of pine wood and comprising oxidized resin acids, oxidized terpenes, polyphenols and polymerized terpenes.

2. A transformer coil including windings of insulated conductive material impregnated and bound with a pine wood pitch obtained by the extraction of pine wood and comprising oxidized resin acids, oxidized terpenes, polyphenols and polymerized terpenes.

3. In combination, an electrical conductor and an insulating material therefor which is impregnated with a pine wood pitch obtained by the extraction of pine wood and comprising oxidized resin acids, oxidized terpenes, polyphenols, and polymerized terpenes.

4. In combination, an electrical conductor and an insulating material therefor comprising asphalt and a pine wood pitch obtained by the extraction of pine wood and comprising oxidized resin acids, oxidized terpenes, polyphenols, and polymerized terpenes.

5. In combination, an electrical conductor and an insulating material therefor comprising castor oil and a pine wood pitch obtained by the extraction of pine wood and comprising oxidized resin acids, oxidized terpenes, polyphenols, and polymerized terpenes.

6. In combination, an electrical conductor and an insulating material therefor which is impregnated with a composition comprising 10 parts by weight of asphalt and 90 parts by weight of a pine wood pitch obtained by the extraction of pine wood and comprising oxidized resin acids, oxidized terpenes, polyphenols, and polymerized terpenes.

7. In combination, an electrical conductor and an insulating material therefor which is impregnated with a composition comprising 10 parts by weight of castor oil and 90 parts by weight of a pine wood pitch obtained by the extraction of pine wood and comprising oxidized resin acids, oxidized terpenes, polyphenols, and polymerized terpenes.

8. In combination, an electrical conductor and an insulating material therefor comprising a pine wood pitch obtained by the extraction of pine wood and heat-treating to prevent foaming thereof, and comprising oxidized resin acids, oxidized terpenes, polyphenols, and polymerized terpenes.

JOHN M. DE BELL.